

Patented June 21, 1932

1,864,107

# UNITED STATES PATENT OFFICE

WILLIAM H. WALTER, OF CYNWYD, PENNSYLVANIA

## PROCESS OF MAKING CORES

No Drawing.

Application filed January 20, 1931. Serial No. 510,057.

Heretofore in making cores for molding metal castings for foundry work it has been found to be the most practical method, as far as known, to use as a binder for the core sand substances such as oil or molasses in the smaller cores while in large cores flour was often used, the sand being mixed with the binder and packed in a core-box, the core reinforced when necessary by chaplets and stiffeners, then vented and placed in an oven to bake, the time required to bake the core being in proportion to its size, some very small cores baking in, say, half an hour while others would remain in the oven over night or longer.

This baking process entailed an unnecessary expense and delay, and in making certain types of castings, the cores were not strong enough to withstand rough handling and broke or became chipped and rendered unfit for use.

The present process or method has in view the provision of a core which does not require baking, is self-venting, and which at the same time is harder and more rugged than baked cores of the old type and does not require chaplets or stiffeners for reinforcing purposes.

The present method consists in making a binding agent by mixing a combustible or inflammable compound such as a solution of celluloid with a volatile solvent such as acetone, butanol, etc., forming a paste. The consistency of the paste is preferably such that it has a very slight tendency to flow and at the same time can be readily handled with a paddle or the like. This binder paste is then mixed with a suitable grade of core sand in the proportion of from ten to twenty-five percent of paste to the amount of sand required to make the core.

The solvent will evaporate to such an extent by air drying only and without the use of heat or baking, that cores of about one inch in thickness can be handled roughly in approximately one-half hour and may be used in a mold within two hours after being made; while the celluloid content of the binder completely burns away during the casting operation so that the core sand flows

freely from cored holes and may be re-claimed.

Cores made with this type of binder are hard and rugged and capable of standing rough usage, maintaining their form over a long span between prints without the use of chaplets or stiffeners. Furthermore, this process produces a porous core which is self-venting.

What I claim is:—

1. The process of making cores of metal castings, which consists in mixing a solution of celluloid with a volatile solvent such as acetone or butanol to form a paste, and mixing the paste with core sand in the proportion of from ten to twenty-five percent of paste to sand.

2. The process of making sand articles such as cores for metal castings, which consists in mixing a solution of celluloid with a volatile solvent to form a binder, and mixing said binder with sand, then shaping said article from said mixture and permitting said solvent to evaporate to set said mixture and form a rigid structure.

3. As an article of manufacture, a rigid sand article composed of sand mixed with a solution of celluloid and a volatile solvent, the sand predominating materially over the celluloid and solvent, and the article being air-dried to evaporate the major portion of the solvent.

In testimony whereof, I have hereunto set my hand.

WILLIAM H. WALTER. 85

90

95

100